

1

2,773,045

## WAX COMPOSITIONS AND SHEET MATERIALS COATED THEREWITH

Linton E. Simerl, Menasha, Alfred M. Heald, Neenah, and George P. Mueller, Appleton, Wis., assignors to Marathon Corporation, Rothschild, Wis., a corporation of Wisconsin

No Drawing. Application February 20, 1951,  
Serial No. 211,968

10 Claims. (Cl. 260—28.5)

This invention relates to wax compositions and more particularly to wet wax coatings and sheet materials coated therewith.

In the manufacture of packaging materials it is the practice to coat a base sheet such as paper, paperboard, cartons, plastic and foil sheets and the like with coating compositions to provide a packaging material with protective properties for the articles packaged. Waxes, particularly petroleum hydrocarbon waxes, i. e., paraffin and microcrystalline wax, are widely used in providing protective coatings for food packaging materials. These waxes are often modified by the addition of other materials which improve the coating for other purposes than the protective function of the coating. For example, in making bread wrappers, paraffin wax is generally used as a coating to provide a protective water-vapor barrier. However, the wax coating also is the medium whereby the wrapper can be heat-sealed and, hence, the seal strength of the coating is very important. Furthermore, since the bread wrapper becomes an advertising or display medium, its gloss and gloss retention properties become an important consideration. It is important that the wax should not come off in handling, i. e., scuff off, so as to become a nuisance to purchasers of the bread. It is very important that the bread wrapper should have low surface friction, i. e., low drag or high slip, so as to function more readily in automatic packaging equipment. It is also important that the coated sheets do not block or stick together, particularly in rolls, under any temperature conditions likely to be encountered in handling. In other types of packaging one or more of the above properties is usually necessary or desirable.

Additives for waxes which are presently available often improve one property to the detriment of another. For example, polyisobutylene or rubber may be added to wax to improve its heat-sealing properties; but at the same time the blocking characteristic, i. e., the tendency for the waxed sheets to stick to each other, is adversely affected. Furthermore, the addition of many wax additives result in an increase in viscosity. If the viscosity is raised above that value at which it can be applied by the usual commercial coating equipment and methods at conventional rates of production, the increase in the cost of manufacture resulting would discourage the use of the additive. For example, a wax composition for making waxed papers and paperboard cartons by conventional wet waxing methods should not be more than 100 centistokes at 210° F. (A. S. T. M. D-445-46T method B) and preferably should have a viscosity of less than about 50 centistokes at 210° F.

It is an object of this invention to provide an improved wax composition for producing waxed packaging materials and particularly heat-sealable materials. It is a further object to provide a wax composition modified by a critical minimum amount of a wax additive to improve heat sealing properties of waxes without impairing blocking, gloss, and slip properties and yet a further object to

2

provide such compositions in which these properties are improved. It is yet a further object to provide a wax composition having a novel combination of wax additives having unique seal strength in relation to the seal strength properties contributed by any of the additives alone. It is still another object to provide heat-sealable waxed sheet materials having improved slip properties. Other objects and advantages will be apparent from the following description of our invention.

We have discovered that certain solid alcohols when added to hydrocarbon waxes, particularly petroleum hydrocarbon waxes, such as paraffin wax and microcrystalline wax, greatly improve the seal strength of the wax and make it more suitable for coating or laminating sheet materials such as paper, paperboard, cellophane, plastic films, and the like. We have further found that small amounts within a critical range, produce a peak value in the seal strength, thus making our composition very economical. The solid alcohols we use are wax-like in character and are sometimes referred to as alcohol-waxes. Prior to our invention the unique effect on the seal strength of wax compositions containing alcohol-waxes had never been appreciated, and particularly the critical range of amounts which we have discovered to be most effective has never, to our knowledge, heretofore been known or disclosed.

The alcohol-waxes which we use in our composition are in general solid aliphatic alcohols, particularly monohydric alcohols, having a melting point above the melting point of the wax or waxes to which they are added. They have a molecular weight in excess of about 500 and preferably 1500. Our preferred alcohol-waxes have a melting point in the range of about 210° F. to about 240° F. (A. S. T. M. D87-42) for an average molecular weight in the range of about 2000 to about 3000 by the Staudinger method. These preferred waxes are, we believe, solid tertiary alcohols, and more specifically dimethyl alkyl carbinol. These preferred waxes are particularly unique in their effect in petroleum waxes. This effect is most evident in compositions which are comprised of at least 90% by weight of petroleum wax and not more than 5% by weight of alcohol-wax. Our preferred tertiary alcohol-waxes are described in United States Patent 2,504,400 as the product of the polymerization of ethylene in the presence of isopropanol and a hydrogen peroxide catalyst. They are believed to have the formula—



where  $\text{R}_1$  and  $\text{R}_2$  are methyl groups and  $\text{R}_3$  is a  $\text{CH}_3-(\text{C}_2\text{H}_4)_n$  where the average value for  $n$  is in the range of about 60 to 100. An alcohol-wax prepared by the process of the above patent of this general formula and having an average molecular weight of about 2100 is available on the market under the trade name Alcowax. It is a product of the Semet-Solvay division of Allied Chemical & Dye Corporation. Though our invention shall hereinafter be described by examples of Alcowax as our alcohol-wax, it is to be understood that other alcohol-waxes of the same general formula are to varying degrees applicable wherein  $\text{R}_1$  and  $\text{R}_2$  are alkyls, such as ethyl, propyl, butyl, etc. and for  $\text{R}_3$ ,  $n$  has an average value greater than about 20. Our preferred alcohols are symmetrical, that is,  $\text{R}_1$  and  $\text{R}_2$  are the same group.

Our improved compositions when coated on sheet materials provide, in addition to seal strength, an excellent combination of gloss, scuff, viscosity and blocking characteristics not heretofore available with any mixture of

wax and wax additives. Furthermore, our compositions are economically desirable. We have found that in general the addition of not more than 5% by weight and preferably about .25% to less than 5% of alcohol-wax, and, specifically Alcowax, to petroleum waxes, will yield a higher seal strength than greater or lesser amounts. The addition of amounts in the range of about 1% to about 2% by weight will in addition provide considerably improved blocking, gloss, scuff and slip characteristics. These critical amounts, since they are small, mean that our compositions are not only low cost, but are also, due in part to the moderate molecular weight of the alcohol-waxes, of low viscosity which makes them well suited for conventional wet waxing methods. Furthermore, in conventional wet waxing, as pointed out above, the lower the viscosity of the wax composition, the higher the production rate, hence, a further cost savings.

In the following tables are set forth the physical properties of a number of examples of paper sheets waxed with wax compositions containing various hydrocarbon waxes and different amounts of Alcowax. The grade of Alcowax used has a melting point of 219° F.-221° F. and a penetration of about .25 mm. at 75° F. as determined on a Kreb's penetrometer, using an ASTM needle, 200 gms. load applied for 5 sec. (Our alcohol-waxes may have penetration values up to .5 mm. and even as high as 1 mm.) Each of the Examples 1-47 was prepared by melting the components together and then surface waxing a bleached sulfate-sulfite paper having a basis weight of 25# per ream (2'x3'-500 sheets) in the conventional manner to obtain about 4 to 6 pounds of surface wax composition per ream. The blocking temperature indicated is the minimum temperature at which coated sheets will block, i. e., stick together sufficiently to prevent separation without disruption of the coating, with the coating face to face when held for 16 hours under a pressure of 0.28 lb. per sq. in. The seal is measured on a Socony-Vacuum Oil Company seal tester, which determines in grams per inch of width of the sheet tested the yield force at 73° F. of two sheets adhered in face to face relation. The "fast" value means that the test pieces were adhered by laminating the two sheets by wrapping them around a roll, steam heated to 210° F., at a speed of 50 ft. per minute and under a tension of about 2 lbs. per sq. in., and then passing the sample at the same speed through a water bath at 61° F. The "slow" value means that the test pieces were cooled in a stream of air at room temperature while traveling at a speed of 10 feet per minute. These seal values bracket the values for seal strength obtainable under commercial sealing conditions, such as in wrapping machines.

TABLE I

Effect of Alcowax on 130/32° F. paraffin wax

| Example | Alcowax, Percent By Weight | Blocking Point, °F. | Seal at 73° F., Grams/in. |      |
|---------|----------------------------|---------------------|---------------------------|------|
|         |                            |                     | Fast                      | Slow |
| 1.      | 0                          | 95                  | 100                       | 23   |
| 2.      | 0.25                       | 105                 | 184                       | 77   |
| 3.      | 0.5                        | 105                 | 218                       | 112  |
| 4.      | 0.75                       | 120                 | 181                       | 115  |
| 5.      | 1.0                        | 135                 | 218                       | 121  |
| 6.      | 1.5                        | 125                 | 254                       | 157  |
| 7.      | 2.0                        | 125                 | 200                       | 164  |
| 8.      | 5.0                        | 130                 | 236                       | 115  |
| 9.      | 10.0                       | 130                 | 184                       | 45   |
| 10.     | 20.0                       | 130                 | 73                        | 53   |

From the above examples it will be seen that paraffin wax compositions modified with up to about 5%, and more particularly with about 0.5% to about 2% Alcowax, have the best seal strength properties. It is further seen that the blocking point sharply increases for

compositions having more than about 0.5% Alcowax. Compositions containing Alcowax in the range of about 1% to about 2% are excellent in respect of both seal strength and blocking. A sheet waxed with these compositions, e. g., Examples 5, 6, and 7, makes a very improved wrapping material, such as, a bread wrapper, plain waxed paper, food overwrap, etc., not only because of the improved blocking and seal characteristics but also because these advantages are obtained with an improvement in the gloss, scuff and slip characteristics. For example, we found the sheets of Examples 5, 6, and 7 show only slight scuff whereas that of Example 1 is great.

Table II illustrates substantially the same results when Alcowax is added to a slightly higher melting point paraffin wax.

TABLE II

Effect of Alcowax on 135/37° F. paraffin wax

| Example | Alcowax, Percent By Weight | Blocking Point, °F. | Seal at 73° F., Grams/in. |      |
|---------|----------------------------|---------------------|---------------------------|------|
|         |                            |                     | Fast                      | Slow |
| 11.     | 0                          | 110                 | 78                        | 17   |
| 12.     | 0.25                       | 110                 | 167                       | 45   |
| 13.     | 0.5                        | 110                 | 192                       | 94   |
| 14.     | 1.0                        | 130                 | 204                       | 116  |
| 15.     | 2.0                        | 135                 | 110                       | 39   |
| 16.     | 5.0                        | 135                 | 110                       | 58   |
| 17.     | 10.0                       | 135                 | 89                        | 51   |
| 18.     | 20.0                       | 135                 | 73                        | 32   |

Here it is seen that the seal strength is sharply improved using as little as .25% Alcowax to about 1% and even up to about 5%. The blocking point increases at about 1% in addition to the increase in seal strength. We further found that there is no significant change in the gloss up to about 5% and the scuff characteristics are improved at .25% and markedly at 1%.

Tables III, IV, V, and VI below illustrate the effect of small additions of Alcowax on various microcrystalline and paraffin hydrocarbon wax blends.

TABLE III

Effect of Alcowax on 20% 140/145° F. microcrystalline wax<sup>1</sup> 80% 135/37° F. paraffin wax

| Example | Alcowax, Percent By Weight | Blocking Point, °F. | Seal at 73° F., Grams/in. |      |
|---------|----------------------------|---------------------|---------------------------|------|
|         |                            |                     | Fast                      | Slow |
| 19.     | 0                          | 115                 | 71                        | 15   |
| 20.     | 0.5                        | 115                 | 115                       | 80   |
| 21.     | 1.0                        | 135                 | 141                       | 97   |
| 22.     | 2.0                        | 120                 | 137                       | 97   |
| 23.     | 3.0                        | 120                 | 143                       | 71   |
| 24.     | 5.0                        | 120                 | 68                        | 60   |

<sup>1</sup> Produced and sold by Shell Oil Co.

TABLE IV

Effect of Alcowax on 35% 140/145° F. microcrystalline wax<sup>1</sup> 65% 135/37° F. paraffin wax

| Example | Alcowax, Percent By Weight | Blocking Point, °F. | Seal at 73° F., Grams/in. |      |
|---------|----------------------------|---------------------|---------------------------|------|
|         |                            |                     | Fast                      | Slow |
| 25.     | 0                          | 110                 | 121                       | 15   |
| 26.     | 0.5                        | 115                 | 143                       | 80   |
| 27.     | 1.0                        | 120                 | 132                       | 92   |
| 28.     | 2.0                        | 120                 | 137                       | 104  |
| 29.     | 3.0                        | 120                 | 137                       | 79   |
| 30.     | 5.0                        | 120                 | 80                        | 43   |

<sup>1</sup> Produced and sold by Shell Oil Co.

5  
TABLE V

Effect of Alcowax on 20% Warco 155° F. microcrystalline wax<sup>1</sup>—80% 135/37° F. paraffin

| Example | Alcowax, Percent By Weight | Blocking Point, °F. | Seal at 73° F., Grams/in. |      | 15 |
|---------|----------------------------|---------------------|---------------------------|------|----|
|         |                            |                     | Fast                      | Slow |    |
| 31      | 1                          | 135                 | 302                       | 149  |    |
| 32      | 2                          | 135                 | 254                       | 185  |    |
| 33      | 3                          | 135                 | 322                       | 110  |    |
| 34      | 5                          | 135                 | 309                       | 62   |    |

<sup>1</sup> Produced and sold by Warwick Wax Co.

TABLE VI

Effect of Alcowax on 20% 145/47° F. microcrystalline wax<sup>1</sup>—80% 135/37° F. paraffin

| Example | Alcowax, Percent By Weight | Blocking Point, °F. | Seal at 73° F., Grams/in. |      | 30 |
|---------|----------------------------|---------------------|---------------------------|------|----|
|         |                            |                     | Fast                      | Slow |    |
| 35      | 1                          | 135                 | 323                       | 141  |    |
| 36      | 2                          | 135                 | 324                       | 176  |    |
| 37      | 3                          | 135                 | 323                       | 131  |    |
| 38      | 5                          | 135                 | 250                       | 72   |    |

<sup>1</sup> Produced and sold by Quaker State Oil Refining Corp.

With each different wax blend it is seen that with additions of Alcowax within the range from about .5% to about 3%, a peak seal is obtained. It further appears that in general a greater improvement is provided by less than 5% additions of Alcowax than by larger amounts. It is further seen that in the range of about 1% to about 2% the best results are obtained as was the case with paraffin wax. In every example containing Alcowax we found that the gloss, and scuff characteristics were maintained or improved and slip definitely improved. Microcrystalline wax has heretofore been blended with paraffin to improve seal strength but such compositions have considerably greater drag or poorer slip than paraffin wax alone. Additives, known heretofore, that would improve the slip properties reduced the seal strength, hence offsetting the advantages of the microcrystalline wax. The compositions in Tables III and IV are therefore, particularly unique for their slip properties and those of Tables V and VI are particularly desirable because of slip and very high seal strength.

Table VII illustrates the effect of Alcowax on a type of wax which is not strictly a paraffin wax because it has some characteristics of a microcrystalline wax, namely, smaller crystal structure, increased tack or stickiness, and high surface friction. It resembles the blends of the previous tables, which may be considered as blends of n-paraffinic, iso-paraffinic and naphthenic hydrocarbons, but is distinct in that the iso-paraffinic and naphthenic components are of lower average molecular weight than is found in microcrystalline waxes. In this wax the iso-paraffinic and naphthenic material, which comprises about 30% by weight of the wax, has the same boiling end point as the n-paraffinic components. These waxes are obtained from high boiling lubricating oil cuts produced by the vacuum distillation of crude oil and have a boiling range of from about 300° F. to about 700° F. at 1 mm. Hg pressure. These waxes in general have melting points of about 140° F. to about 170° F.

6  
TABLE VII

Effect of Alcowax on Aristowax<sup>1</sup> 143/50° F.

| Example | Alcowax, Percent By Weight | Blocking Point, °F. | Seal at 73° F., Grams/in. |      |
|---------|----------------------------|---------------------|---------------------------|------|
|         |                            |                     | Fast                      | Slow |
| 39      | 0                          | 115                 | 101                       | 19   |
| 40      | 0.25                       | 135                 | 97                        | 42   |
| 41      | 0.5                        | 135                 | 92                        | 67   |
| 42      | 0.75                       | 135                 | 110                       | 87   |
| 43      | 1.0                        | 135                 | 167                       | 86   |
| 44      | 2.0                        | 135                 | 167                       | 77   |
| 45      | 5.0                        | 135                 | 42                        | 45   |
| 46      | 10.0                       | 135                 | 54                        | 63   |
| 47      | 20.0                       | 135                 | 55                        | 44   |

<sup>1</sup> Produced and sold by Union Oil Co. of California.

From the above it is seen that as little as about .25% Alcowax improves the blocking and seal characteristic of the wax of Table VII when compared to the control or the example containing 5% Alcowax. Here the range of about .75% to about 2% is preferred which corresponds closely to the preferred range for the compositions in the preceding tables. These compositions, we have found, also have good gloss, scuff, and slip properties. Heretofore the poor slip properties of compositions containing this type of wax have limited its use.

Table VIII below illustrates the seal strength at two different temperatures of compositions of Alcowax and the microcrystalline wax used in the blend of Table VI which is a wax from a Pennsylvania crude. The seal strengths shown are the "fast" values at the temperatures indicated and the coated base sheet is #300 MAT-2 cellophane.

TABLE VIII

Effect of Alcowax on 145/47° F. microcrystalline wax<sup>1</sup>

| Example | Percent Alcowax | Seal—Grams/in.—Fast |        |
|---------|-----------------|---------------------|--------|
|         |                 | 73° F.              | 45° F. |
| 48      | 0               | 744                 | 754    |
| 49      | 0.25            | 810                 | 981    |
| 50      | 0.5             | 840                 | 1,004  |
| 51      | 0.75            | 810                 | 1,017  |
| 52      | 1               | 810                 | 1,017  |
| 53      | 1.5             | 1,051               | 1,203  |
| 54      | 2               | 1,190               | 1,203  |
| 55      | 3               | 949                 | 642    |

<sup>1</sup> Produced and sold by Quaker State Refining Corp.

At 73° F. and 45° F. the amounts of Alcowax for improved seal strength are clearly illustrated as being in the general range of .25% to 2% with some improvement even at 3%. It is clearly evident from the results shown by each table above, and particularly, Tables II, VI, and VIII, that amounts of Alcowax in about the same critical ranges in paraffin wax, microcrystalline wax, and a blend of each, will in each case produce a composition having improved seal strength and blocking characteristics.

Polyethylene, which is in commercial use as a wax additive, serves to improve blocking, gloss, scuff resistance, and seal stability, that is, by our definition the ratio of "slow" to "fast" seal values. It does not function, however, as Alcowax, within our critical concentration ranges, to improve the "fast" value as well as the stability and also maintain or improve blocking. In fact with microcrystalline wax, polyethylene reduces the seal strength. Furthermore, the characteristic or property of "slip" which we have used herein to define the degree of friction between the coating and foreign surfaces, such as wrapping machine surfaces, is far superior with Alcowax-wax compositions than with polyethylene-wax compositions. Still a further important advantage of Alcowax over polyethylene as a wax additive is that there is little increase in viscosity in the resulting wax composition particularly within the critical range of percentages.

we prefer. For example, the viscosity of compositions of Table I were less than 9 centistokes at 210° F. In the case of the microcrystalline wax compositions, the viscosities were not in excess of about 20 centistokes at 210° F. Similar polyethylene wax compositions would have considerably higher viscosities.

Alcowax may be used along with other wax additives which may be added in small amounts to obtain certain special properties. Additives, such as rubber, polyisobutylene, polyethylene, rosin and rosin esters, vegetable gums, metal stearates, and plasticizers, such as petro-latum, may be used. In general, however, our preferred compositions will contain at least about 75%, and preferably 90%, hydrocarbon wax and will have a viscosity of less than 100 centistokes at 210° F. and preferably less than 50 centistokes at 210° F.

When polyethylene is used together with Alcowax in wax compositions we have found a totally unexpected improvement in seal strength which indicates a synergistic effect. Table IX below illustrates this. Each example was prepared by coating a paper base sheet to obtain about 4 to 6 pounds per ream of the described composition on the surface as in the examples in the Tables I-VII.

TABLE IX.  
*Effect of combining Alcowax and polyethylene*

| Example | Composition                                                                                                                                                                                                                                                                                                                                                                                                                                                                                                                                                                                                                                                                                                             | Block-ing Point, °F. | Seal at 73° F., Grams/in. |      |
|---------|-------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|----------------------|---------------------------|------|
|         |                                                                                                                                                                                                                                                                                                                                                                                                                                                                                                                                                                                                                                                                                                                         |                      | Fast                      | Slow |
| 56      | [3.5% Polyethylene (7,000 Mol. Wt.)..<br>35.0% 145/47° F. Microcrystalline Wax.<br>61.5% 135/37° F. Paraffin Wax...<br>3.5% Alcowax...<br>35.0% 145/47° F. Microcrystalline Wax.<br>61.5% 135/37° F. Paraffin Wax...<br>1.75% Alcowax...<br>1.75% Polyethylene (7,000 Mol. Wt.)...<br>35.0% 145/47° F. Microcrystalline Wax.<br>61.5% 135/37° F. Paraffin Wax...<br>9% Polyethylene (7,000 Mol. Wt.)...<br>40% 145/47° F. Microcrystalline Wax.<br>51% 135/37° F. Paraffin Wax...<br>9% Alcowax...<br>40% 145/47° F. Microcrystalline Wax.<br>51% 135/37° F. Paraffin Wax...<br>4.5% Alcowax...<br>4.5% Polyethylene (7,000 Mol. Wt.)...<br>40.0% 145/47° F. Microcrystalline Wax.<br>51.0% 135/37° F. Paraffin Wax...] | 115                  | 134                       | 68   |
| 57      |                                                                                                                                                                                                                                                                                                                                                                                                                                                                                                                                                                                                                                                                                                                         | 115                  | 126                       | 60   |
| 58      |                                                                                                                                                                                                                                                                                                                                                                                                                                                                                                                                                                                                                                                                                                                         | 115                  | 147                       | 111  |
| 59      |                                                                                                                                                                                                                                                                                                                                                                                                                                                                                                                                                                                                                                                                                                                         | 125                  | 149                       | 169  |
| 60      |                                                                                                                                                                                                                                                                                                                                                                                                                                                                                                                                                                                                                                                                                                                         | 115                  | 162                       | 144  |
| 61      |                                                                                                                                                                                                                                                                                                                                                                                                                                                                                                                                                                                                                                                                                                                         | 130                  | 259                       | 208  |

A comparison of Examples 56 and 57 with 58 and of Examples 59 and 60 with 61 shows that the combination of polyethylene and Alcowax produces a greater seal strength than the same percentage of either additive alone. This unique result may in part be explained by the fact that in Examples 58 and 61 the amount of Alcowax is within our preferred range; about 1% to 2% in the case of Example 58 and of less than 5% in case of Example 61. Whatever the explanation, however, these examples further illustrate that desirable compositions can be produced which comprise from about .5% to less than about 5% by weight of Alcowax, about 1% to about 5% by weight of solid polyethylene, and the balance, or at least about 75% by weight, a mixture of a paraffin and microcrystalline wax.

Compositions of Alcowax, in our critical amounts, and paraffin wax, alone or with microcrystalline wax, when coated on paper, paperboard, regenerated cellulose and plastic films, result in materials extremely well suited for heat-sealing food wraps and containers. Because of the seal strength properties, our compositions, particularly those containing microcrystalline wax, are excellent lami-

nants. Excessive oil in paraffin wax will affect its properties, and the paraffin wax portion of our compositions is therefore of relatively low oil content, i. e., of less than about .75% and preferably about .5% when measured by A. S. T. M. method D-721-43T.

Many other modifications of our improved composition other than those given herein by way of example will occur to those skilled in the art and no limitations are intended by the above examples except such as are contained in the following claims.

We claim:

1. A heat-sealable sheet material comprising a fibrous paper base sheet having a superficial coating comprising a solid polymer of ethylene and isopropanol having the formula



wherein  $\text{R}_1$  and  $\text{R}_2$  are methyl groups and  $\text{R}_3$  is a  $\text{CH}_3-(\text{C}_2\text{H}_4)_n$  group where the average value for  $n$  is in the range of about 60 to 100, said polymer being present in amounts from .25% to 5% by weight and having a molecular weight in the range of from 500 to about 3000 and having a melting point of from about 210° F. to about 240° F., 1% to 5% by weight of solid polyethylene, and 75% to about 98.75% of petroleum wax having a melting point of from about 130° F. to about 170° F.

2. A heat-sealable sheet material comprising a fibrous paper base sheet having a superficial coating comprising a solid polymer of ethylene and isopropanol having the formula



wherein  $\text{R}_1$  and  $\text{R}_2$  are methyl groups and  $\text{R}_3$  is a  $\text{CH}_3-(\text{C}_2\text{H}_4)_n$  group where the average value for  $n$  is in the range of about 60 to 100, having a melting point in excess of 200° F. and a solid polyethylene in about equal proportions, from about 20% to about 50% microcrystalline wax, from about 40% to about 80% paraffin wax, having a melting point of from about 130° F. to about 210° F., said combined polymer and polyethylene having a ratio to the combined paraffin and microcrystalline wax of from 1:28 to about 1:10.

3. A wax composition comprising paraffin wax containing from 0.5 to 10% by weight of a mixture of polyethylene and 40 to 60% by weight based on total polymer of polyethylene having a terminal hydroxyl group, said hydroxylated polyethylene being produced by polymerizing ethylene under 425-475 atmospheres at temperatures between 140° and 200° C. in the presence of isopropanol and hydrogen peroxide.

4. Composition according to claim 3 in which the polyethylene has a molecular weight of 4,000-25,000 and the polyethylene having a terminal hydroxyl group has a molecular weight of about 500-10,000.

5. Composition according to claim 3 in which the polyethylene has a molecular weight of 12,000-13,000 and the polyethylene having a terminal hydroxyl group has a molecular weight of about 2,000.

6. A wax composition comprising paraffin wax containing 1.5 to 2.5% by weight of a mixture of polyethylene and 40 to 60% by weight based on total polymer of polyethylene having a terminal hydroxyl group, said hydroxylated polyethylene being produced by polymerizing ethylene under 425-475 atmospheres at temperatures between 140° and 200° C. in the presence of isopropanol and hydrogen peroxide.

7. Composition according to claim 6 in which the polyethylene has a molecular weight of 4,000-25,000 and the polyethylene having a terminal hydroxyl group has a molecular weight of about 500-10,000.

8. Composition according to claim 6 in which the poly-

ethylene has a molecular weight of 12,000-13,000 and the polyethylene having a terminal hydroxyl group has a molecular weight of about 2,000.

9. Composition according to claim 8 in which the amount of the total polymers is about 2.5% by weight. 5

10. A heat-sealable sheet material comprising a fibrous paper base sheet having a superficial coating comprising a solid polymer of ethylene and isopropanol having the formula



wherein R<sub>1</sub> and R<sub>2</sub> are methyl groups and R<sub>3</sub> is a CH<sub>3</sub>-(C<sub>2</sub>H<sub>4</sub>)<sub>n</sub> group where the average value for n is in the range of about 60 to 100, said polymer being present in amounts by weight from 0.25% to about 5%, from about 1% to about 5% of solid polyethylene, from about 35% to about 40% of microcrystalline wax, and from about 50% to about 60% paraffin wax having a melting point of from about 130° to about 210° F. 15

References Cited in the file of this patent

UNITED STATES PATENTS

|           |                 |               |
|-----------|-----------------|---------------|
| 1,950,814 | Pungs et al.    | Mar. 13, 1934 |
| 2,350,292 | Sermattei       | May 30, 1944  |
| 2,361,582 | Adams et al.    | Oct. 31, 1944 |
| 2,402,137 | Hanford et al.  | June 18, 1946 |
| 2,409,683 | Howk et al.     | Oct. 22, 1946 |
| 2,504,270 | MacLaren et al. | Apr. 18, 1950 |
| 2,504,400 | Erchak          | Apr. 18, 1950 |
| 2,551,087 | Barnhart et al. | May 1, 1951   |
| 2,560,773 | Lovell          | July 17, 1951 |
| 2,582,037 | Hyde            | Jan. 8, 1952  |
| 2,712,534 | Erchak          | July 5, 1955  |

FOREIGN PATENTS

|         |               |               |
|---------|---------------|---------------|
| 621,923 | Great Britain | Apr. 22, 1949 |
|---------|---------------|---------------|

OTHER REFERENCES

The Chemistry and Technology of Waxes, Waith Reinbold Publishing Company, New York, New York, 1947.